

## UNITED STATES PATENT OFFICE

2,056,386

PROTECTION OF HEAT RESISTANT ALLOYS  
AGAINST CARBURIZATION

Adrien Cambren, Ottawa, Ontario, Canada

No Drawing. Application December 26, 1934.  
Serial No. 759,232

6 Claims. (Cl. 91—70)

This invention relates to the protection of reaction chambers, formed of heat resisting alloys, where these are used for carrying out reactions in which the metal is subjected to a carburizing atmosphere at high temperatures.

It has been found that when such chambers or tubes, which are normally resistant to air oxidation at temperatures of, say, 950° C., are used for purposes, such as the pyrolysis of hydrocarbon gases or the vapour-phase cracking of petroleum fractions, the metal becomes covered with a film of carbon. When air is passed through the tube to remove the carbon film the metal becomes coated with a loose deposit of a mixture of the oxides of the metals of the alloy. In the case of chromium-nickel or high chromium alloys the coating is of a brick red colour.

The formation of these coatings on the surfaces of the reaction tubes has a pronounced effect on the course of the reactions and reduces the rate of heat transfer through the walls as well as the capacity of the tubes. The presence of the oxides causes the surfaces to become active in promoting carbon deposition and the increased rate at which the carbon deposits necessitates more frequent blowing of the tubes with air to remove the carbon. For example, it has been reported that tubes made from an alloy containing 18% chromium and 8% nickel and used for the pyrolysis of hydrocarbon gases at about 900° C. required blowing with air every 10 to 12 hours to remove the carbon deposit, and that the tubes failed after less than 50 hours' use, the failure being due to carburization.

The object of the present invention is to overcome these defects, to increase the useful life of the tubes and to avoid the blocking of the tube, as well as the lowering of the rate of heat transfer through the wall of the tubes.

The invention contemplates preventing direct contact between the heat resistant alloys of such tubes and the carbon, so that the tubes may be heated alternately under carburizing and oxidizing conditions without decrease in their heat resistance or apparent alteration in the structure of the alloys. This is accomplished by covering the surface of the metal exposed to the reactions with a protective coating of inert substances. The coating may be applied by brushing, spraying or dipping, after which it is fused on the metal by heating to temperatures around 750° to 850° C.

A thin continuous film of  $B_2O_3$  forms such a protective coating.  $Cr_2O_3$  may be mixed with  $H_3BO_3$  in the proportions of one part of the former with one to four parts of the latter. Boric

anhydride is the equivalent of boric acid. These materials are made up into a thin paste by suspending them in water or alcohol for application to the metal surfaces. The  $Cr_2O_3$  may be replaced in whole or in part by other refractory oxides, such as  $BeO$ ,  $MgO$ ,  $Al_2O_3$ . When treating high chromium alloys, such as those containing 28% of chromium, the  $B_2O_3$  may be replaced in whole or in part by  $V_2O_5$  and some of the  $Cr_2O_3$  may be present in the form of chromite.

With alloys, such as those containing 18% chromium and 8% nickel, care must be taken not to subject them to too great and sudden changes of temperature, since this has a tendency to loosen the coating, owing to the relatively high coefficients of thermal expansion of such alloys. With high chromium alloys, such as those containing over 20% chromium, the so-coated metals may be heated to temperatures as high as 950°C. and then cooled to room temperature without affecting the adherance or continuity of the coating or altering its protective action.

The invention has particular utility in the pyrolysis of hydrocarbon gases and in the vapour-phase cracking of petroleum fractions at temperatures about 700°-950° C. The protective coating prevents the carburization of the metal of the reaction tubes and the results which follow such action, maintains the normal rate of heat conductivity of the metal and eliminates the catalytic effect on carbon deposition of the oxide deposits which form on unprotected metals of this character.

I claim:

1. Heat resistant chromium alloys having a surface coating consisting of a continuous film consisting essentially of one of the group consisting of  $B_2O_3$  and  $V_2O_5$ , said film being fused on the surface of the alloy.

2. Heat resistant alloys having a surface coating consisting of a continuous film of a mixture of one of the group consisting of  $B_2O_3$  and  $V_2O_5$  and one of the refractory group consisting of  $Cr_2O_3$ ,  $BeO$ ,  $MgO$  and  $Al_2O_3$ , said film being fused on the surface of the alloy.

3. Chromium alloys having a coating consisting of a continuous film consisting of  $B_2O_3$  and  $Cr_2O_3$ , said film being fused on the surface of the alloy.

4. A method of protecting heat resistant alloys against carburization during pyrolysis of hydrocarbon gases or vapours which comprises applying a continuous coating consisting essentially of  $B_2O_3$  to the surface of the alloy and fusing the coating thereto.

5. A method as defined in claim 4 wherein one of the group of refractory oxides consisting of  $\text{Cr}_2\text{O}_3$ ,  $\text{BeO}$ ,  $\text{MgO}$  and  $\text{Al}_2\text{O}_3$  is combined with the  $\text{B}_2\text{O}_3$ .
- 5 6. A method of protecting chromium alloys against carburization during pyrolysis of hydro-carbon gases or vapour-phase cracking of petro-

leum fractions which comprises forming a mixture consisting essentially of  $\text{Cr}_2\text{O}_3$  and  $\text{B}_2\text{O}_3$ , applying a continuous film of the mixture to the alloy and heating the coated alloy at about 750° to 850° C. to fuse the film on the alloy.

ADRIEN CAMBRON.